



US009340733B2

(12) **United States Patent**  
**Marchand et al.**

(10) **Patent No.:** **US 9,340,733 B2**  
(45) **Date of Patent:** **May 17, 2016**

(54) **PROCESS FOR HYDRODESULPHURATION OF GASOIL CUTS USING A CATALYST BASED ON HETEROPOLYANIONS TRAPPED IN A MESOSTRUCTURED SILICA SUPPORT**

(71) Applicants: **IFP ENERGIES NOUVELLES, Rueil-Malmaison (FR); CENTRE NATIONAL DE LA RECHERCHE SCIENTIFIQUE, Paris (FR)**

(72) Inventors: **Karin Marchand, Allemagne (DE); Alexandra Chaumonnot, Lyons (FR); Audrey Bonduelle, Francheville (FR); Magalie Roy-Auberger, Nivolas-Vermelle (FR); Veronique Dufaud, Villeurbanne (FR); Frederic Lefebvre, Beaufort (FR); Manuela Bader, Rennes (FR); Susana Lopes Silva, Lyons (FR)**

(73) Assignees: **CENTRE NATIONAL DE LA RECHERCHE SCIENTIFIQUE, Paris (FR); IFP ENERGIES NOUVELLES, Rueil-Malmaison (FR)**

(\*) Notice: Subject to any disclaimer, the term of this patent is extended or adjusted under 35 U.S.C. 154(b) by 117 days.

(21) Appl. No.: **14/182,698**

(22) Filed: **Feb. 18, 2014**

(65) **Prior Publication Data**

US 2014/0231310 A1 Aug. 21, 2014

**Related U.S. Application Data**

(63) Continuation of application No. 13/996,754, filed as application No. PCT/FR2011/000652 on Dec. 15, 2011, now abandoned.

(30) **Foreign Application Priority Data**

Dec. 22, 2010 (FR) ..... 10 05028

(51) **Int. Cl.**

*C10G 45/04* (2006.01)  
*C10G 45/08* (2006.01)  
*C10G 45/06* (2006.01)  
*C10G 69/04* (2006.01)  
*C10G 45/00* (2006.01)  
*C10G 45/02* (2006.01)

(52) **U.S. Cl.**

CPC ..... *C10G 45/08* (2013.01); *C10G 45/04* (2013.01); *C10G 45/06* (2013.01); *C10G 69/04* (2013.01); *C10G 2300/202* (2013.01)

(58) **Field of Classification Search**

CPC ..... B01J 27/186; B01J 27/188; B01J 27/19; B01J 27/195; B01J 27/198

See application file for complete search history.

(56) **References Cited**

**U.S. PATENT DOCUMENTS**

|                  |         |                               |
|------------------|---------|-------------------------------|
| 7,737,071 B2     | 6/2010  | Kiriyama et al.               |
| 2004/0186013 A1  | 9/2004  | Iwata et al.                  |
| 2008/0017551 A1  | 1/2008  | Kiriyama et al.               |
| 2008/0020926 A1* | 1/2008  | Guillaume et al. .... 502/314 |
| 2008/0314797 A1* | 12/2008 | Sinclair et al. .... 208/49   |
| 2009/0171123 A1* | 7/2009  | Glaser et al. .... 568/376    |
| 2011/0230691 A1* | 9/2011  | Bonduelle et al. .... 585/266 |

**FOREIGN PATENT DOCUMENTS**

EP 1733787 A1 12/2006

**OTHER PUBLICATIONS**

Corma, A. et al. (1995). *Journal of Catalysis*, 153, 25-31.\*  
International Search Report for PCT/FR2011/000652 (Feb. 14, 2012).

A. Rives et al., "Silica and Alumina Impregnated with Dimethylformamide Solutions of Molybdochosphoric or Tungstophosphoric Acids for Hydrotreatment Reactions", *Catalysis Letters*, vol. 71, No. 3-4 (2001) pp. 193-201.

X.M. Yan et al., "Synthesis and Catalytic Properties of Mesoporous Phosphotungstic Acid/SiO<sub>2</sub> in a Self-Generated Acidic Environment by Evaporation-Induced Self-Assembly", *Materials Research Bulletin*, vol. 42 (2007) pp. 1905-1913.

C. Lamonier et al., "Molybdochalcobaltate Cobalt Salts: New Starting Materials for Hydrotreating Catalysts", *Applied Catalysis B: Environmental*, vol. 70 (2007) pp. 548-556.

X.M. Yan et al., "Oxidative Desulfurization of Diesel Oil Using Mesoporous Phosphotungstic Acid/SiO<sub>2</sub> as Catalyst", *Journal of the Chinese Chemical Society*, vol. 54 (2007) pp. 911-916.

X.M. Yan et al., "Synthesis and Characterization of Mesoporous Phosphotungstic Acid/TiO<sub>2</sub> Nanocomposite as a Novel Oxidative Desulfurization Catalyst", *Journal of the Molecular Catalysis A: Chemical*, vol. 304 (2009) pp. 52-57.

C. Martin "Catalyseurs D'Hydrodesulfuration Prepares a Partir D'Heteropolyanions De Type Anderson", *Universite Des Sciences Et Technologie De Lille* (Oct. 21, 2003) XP002638548.

\* cited by examiner

**Primary Examiner** — Brian McCaig

(74) **Attorney, Agent, or Firm** — Millen White Zelano and Branigan, PC; Csaba Henter; Anthony Zelano

(57) **ABSTRACT**

The invention relates to a process of hydrodesulphuration of at least one gasoil cut implementing a catalyst containing, in its oxide form, at least one metal from group VIB and/or at least one metal from group VIII of the periodic table, present in the form of at least one polyoxometalate of the formula (H<sub>n</sub>X<sub>x</sub>M<sub>m</sub>O<sub>y</sub>)<sup>q-</sup>, said polyoxometalates being present within a mesostructured silicon oxide matrix having a pore size within the range 1.5 to 50 nm and having amorphous walls of thickness within the range 1 to 30 nm, the said catalyst being sulphured before being implemented in the said process.

**13 Claims, No Drawings**

**PROCESS FOR HYDRODESULPHURATION  
OF GASOIL CUTS USING A CATALYST  
BASED ON HETEROPOLYANIONS TRAPPED  
IN A MESOSTRUCTURED SILICA SUPPORT**

The present invention relates to the field of hydrotreatment of hydrocarbon feeds of the gasoil type.

Its main subject is the use of a catalyst in processes enabling the hydrodesulphuration (HDS) of feeds of the gasoil type.

**PRIOR ART**

The increased stringency of motor-vehicle emissions standards in 2009 within the European Union is constraining refiners to greatly reduce the sulphur content of gasoils and gasolines, to a maximum of 10 parts of sulphur per million (ppm) by weight in gasoils on 1 Jan. 2009, as compared with 50 ppm on 1 Jan. 2005 (measured by the ASTM D-4294 method). These constraints translate into a need for new refining facilities or else into a large increase in the isovolumetric activity of hydrotreatment catalysts. These new constraints will also lead to an increased need for hydrogen in refineries, hydrogen being necessary for hydrodesulphuration, hydrodenitrogenation and hydrodearomatisation reactions. Moreover, these new standards are also accompanied by constraints in respect of product quality. Thus, the gasoils must have a good cetane index. The reactions of hydrotreatment of gasoils similarly induce the hydrogenation of aromatic cores contained in the said gasoil cuts, which has the consequence of improving the cetane index of the said final gasoil cut, but can cause an over-consumption of hydrogen if the cetane index already complies with the specifications.

The increased performances of the hydrotreatment of gasoil cuts may be due in part to the choice of method, but in all cases the use of an intrinsically more active catalytic system is very often a key factor. Thus, new methods of preparing hydrotreatment catalysts need to be developed to further improve the performance of these catalysts and to comply with future legislation.

It is generally acknowledged that a hydrotreatment catalyst of high catalytic potential is characterised by an optimised hydro-dehydrogenating function, that is, by an active phase perfectly dispersed at the surface of the support and having a high metal content. Ideally, whatever the nature of the hydrocarbon feed to be treated, the catalyst must be able to demonstrate an accessibility of the active sites to reactants and products of reaction while at the same time developing a larger active surface area, resulting in specific constraints in respect of structure and texture that are specific to the oxide support constituting the said catalysts.

The composition and use of conventional catalysts for the hydrotreatment of hydrocarbon feeds are described well in "Hydrocracking Science and Technology", 1996, J. Scherzer, A. J. Gruia, Marcel Dekker Inc and in the article of B. S. Clausen, H. T. Topsoe, F. E. Massoth, from the work "Catalysis Science and Technology", 1996, volume 11, Springer-Verlag. Thus, these catalysts are generally characterised by the presence of an active phase based on at least one metal from group VIB and/or at least one metal from group VIII of the periodic table of the elements. The most widely-used formulations are of the cobalt-molybdenum (CoMo), nickel-molybdenum (NiMo) and nickel-tungsten (NiW) types. These catalysts can be in bulk, or in the supported state, in which case they include a porous solid of a different nature. In the latter case, the porous support is generally an amorphous or poorly crystallised oxide such as, for example, an alumina,

or an aluminosilicate, optionally combined with a zeolithic or non-zeolithic material. Following preparation, at least one group VIB metal and/or at least one group VIII metal constituting the said catalysts are often in the oxide form. As the form of the said catalysts for the hydrotreatment processes that is active and stable is the sulphured form, these catalysts must undergo a sulphuration step. This may be performed within the unit for the associated process, when it is called sulphuration in-situ, or before the catalyst is fed into the unit, in which case it is called sulphuration ex-situ.

The conventional methods leading to the formation of the active phase of hydrotreatment catalysts consist in a deposition of molecular precursor(s) of at least one group VIB metal and/or at least one group VIII metal onto an oxide support by the technique known as "dry impregnation" followed by the steps of maturation, drying and calcination leading to the formation of the oxidised form of the said metal(s) used. This is followed by the final step of sulphuration which generates the active phase, as mentioned above.

The catalytic performances of hydrotreatment catalysts derived from these "conventional" synthesis protocols have been widely studied. In particular, it has been shown that, when metal contents are relatively elevated, phases refractory to sulphuration appear, which are formed consecutively to the calcination step and are due to a sintering phenomenon (B. S. Clausen, H. T. Topsoe, and F. E. Massoth, from "Catalysis Science and Technology", 1996, volume 11, Springer-Verlag). For example, in the case of catalysts of the CoMo or NiMo type supported on a support of the aluminic nature, these phases refractory to sulphuration are either crystallites of metallic oxides of the formula  $\text{MoO}_3$ ,  $\text{NiO}$ ,  $\text{CoO}$ ,  $\text{CoMoO}_4$  or  $\text{Co}_3\text{O}_4$ , of sufficient size to be detected by DRX, or species of the type  $\text{Al}_2(\text{MoO}_4)_3$ ,  $\text{CoAl}_2\text{O}_4$  or  $\text{NiAl}_2\text{O}_4$ , or both. The three species of type  $\text{Al}_2(\text{MoO}_4)_3$ ,  $\text{CoAl}_2\text{O}_4$  or  $\text{NiAl}_2\text{O}_4$  containing the element aluminium are well-known to the person skilled in the art. They result from the interaction between the alumina support and the precursor salts in solution of the active phase, the chemical manifestation of which is a reaction between  $\text{Al}^{3+}$  ions extracted from the alumina matrix and the said salts to form Anderson heteropolyanions of the formula  $[\text{Al}(\text{OH})_6\text{Mo}_6\text{O}_{18}]^{3-}$ , themselves precursors of phases refractory to sulphuration. The presence of all these species together leads to a not inconsiderable indirect loss of the catalytic activity of the associated hydrotreatment catalyst, because the elements belonging to at least one group VIB metal and/or at least one group VIII metal are not entirely utilised to their maximum potential, since a portion thereof is immobilised in minimally active or inactive species.

The catalytic performances of the conventional hydrotreatment catalysts described above could therefore be improved, notably by developing new methods of preparing these catalysts, which would enable:

- 1) assurance of a good dispersion of the active phase, particularly for elevated metal contents, for example by controlling the size of the particles based on transition metals and maintaining the properties of these particles following heat treatment,
- 2) limitation of the formation of species refractory to sulphuration, for example by achieving a better synergy between the transition metals constituting the active phase and control of the interactions between the active phase and/or its precursors, and the porous support employed,
- 3) assurance of a good diffusion of the reactants and of the reaction products while also maintaining large developed active surface areas, for example by optimising the chemical, textural and structural properties of the porous support.

A number of research pathways regarding the development of new catalysts for hydrotreatment of gasoil cuts have attempted to respond to the needs stated above.

The research conducted by the Applicant thus led to the preparation of hydrotreatment catalysts by modifying the chemical and structural composition of the metallic species that are precursors of the active phases and thus by modifying the interactions between the support and the active phase of the catalyst and/or its oxide precursors. In particular, the work of the Applicant led to the use of the polyoxometalates of the formula given below as specific oxide precursors of the active phase of the catalysts used in the hydrodesulphuration process of gasoil cuts according to the invention.

Moreover, as the oxide support of the catalyst plays a not inconsiderable role in the development of high-performance hydrotreatment catalysts to the extent that it induces modifications of the interactions between the support and the active phase of the said catalyst and/or its oxide precursors, the research work of the Applicant was also directed towards the preparation of hydrotreatment catalysts using oxide supports having particular textural properties.

The Applicant has therefore demonstrated that a catalyst comprising, in its oxide form, at least one active phase precursor in the form of at least one polyoxometalate of the formula  $(H_xX_xM_mO_y)^{q-}$  explained below, trapped actually within a mesostructured silica oxide matrix serving as a support, showed an improved catalytic activity by comparison with catalysts prepared from standard precursors not containing polyoxometalates, the said catalyst being sulphured then implemented in a hydrodesulphuration process of at least one gasoil cut according to the invention.

One aim of the present invention is to provide a hydrodesulphuration process of at least one gasoil cut implementing a catalyst having improved catalytic performances.

Another aim of the present invention is to provide a hydrodesulphuration process of at least one gasoil cut implementing a catalyst having improved catalytic performances, the said process enabling increased hydrodesulphuration activity to be achieved, and the cetane index of the said gasoil cut to be maintained at a high level while keeping the hydrogen consumption of the said process constant.

## SUMMARY OF THE INVENTION

The invention relates to a hydrodesulphuration process of at least one gasoil cut implementing a catalyst comprising, in its oxide form, at least one metal of group VIB and/or at least one metal of group VIII of the periodic table present in the form of at least one polyoxometalate of the formula  $(H_xX_xM_mO_y)^{q-}$ , wherein X is an element selected from phosphorus (P), silicon (Si), boron (B), nickel (Ni) and cobalt (Co), the said element being taken alone, M is one or more element(s) selected from molybdenum (Mo), tungsten (W), nickel (Ni) and cobalt (Co), O is oxygen, H is hydrogen, h is an integer within the range 0 to 12, x is an integer within the range 0 to 4, m is an integer equal to 5, 6, 7, 8, 9, 10, 11, 12 and 18, y is an integer within the range 17 to 72 and q is an integer within the range 1 to 20, the said polyoxometalates being present within a mesostructured silicon oxide matrix having a pore size within the range 1.5 to 50 nm and having amorphous walls of thickness within the range 1 to 30 nm, the said catalyst being sulphured before being implemented in the said process.

## BENEFITS OF THE INVENTION

One of the advantages of the present invention is given by the implementation, in a hydrodesulphuration process of at

least one gasoil cut, of a catalyst having simultaneously the catalytic properties specific to the presence of polyoxometalates and the properties of surface reactivity of the mesostructured silicon oxide matrix in which the said polyoxometalates are trapped. The result of this is therefore innovative properties and interactions between the said polyoxometalates and the mesostructured inorganic silica lattice of the said matrix. These interactions are manifested in an enhanced hydrodesulphuration activity with no significant increase in the hydrogen consumption as compared with the catalysts described in the prior art, this being due in particular to a better dispersion of the active phase owing to the use of a mesostructured silicon oxide matrix in which polyoxometalates are trapped.

In particular, the catalyst described according to the invention enables a final hydrodesulphuration of the gasoil cuts with a reduced hydrogen consumption, for an activity identical to that of current commercially available catalysts.

## DESCRIPTION OF THE INVENTION

The invention relates to a hydrodesulphuration process of at least one gasoil cut.

### Feeds

The feed implemented in the hydrodesulphuration process according to the invention is a sulphur-containing gasoil cut. Gasoil cuts generally have a sulphur content within the range 1 to 5 wt. % in the case of a gasoil cut derived by direct distillation (or "straight-run gasoil") and a sulphur content of more than 300 ppm in the case of a gasoil cut sourced from conversion processes.

The gasoil cuts implemented in the process according to the invention are advantageously selected from the gasoil cuts derived by direct distillation (or "straight-run gasoil") alone or in admixture with at least one cut derived from a coking unit, or at least one cut derived by catalytic cracking (Fluid Catalytic Cracking), or at least one gasoil cut sourced from other conversion processes such as soft hydrocracking or residue hydrotreatment. The gasoil cuts implemented in the process according to the invention are cuts at least 90% of the compounds of which have a boiling point within the range 250° C. to 400° C.

The hydrodesulphuration process of at least one gasoil cut according to the invention is advantageously implemented at a temperature within the range 250° C. to 400° C., preferably 320° C. to 380° C. at a total pressure within the range 2 MPa to 10 MPa and preferably 3 MPa to 9 MPa with a ratio of the volume of hydrogen to volume of hydrocarbon feed within the range 100 to 600 litres per litre and preferably within the range 200 to 400 litres per litre, and at an hourly space velocity (HSV) defined by the ratio of the volumetric flow rate of liquid hydrocarbon feed to the volume of catalyst fed into the reactor within the range 1 to 10 h<sup>-1</sup>, and preferably 2 to 8 h<sup>-1</sup>.

According to the invention, the catalyst used in the said hydrodesulphuration process comprises, in its oxide form, that is to say before having undergone a sulphuration step generating the sulphide active phase, at least one metal of group VIB and/or at least one metal of group VIII of the periodic table present in the form of at least one polyoxometalate of the formula  $(H_xX_xM_mO_y)^{q-}$  explained above, the said polyoxometalates being present within a mesostructured silicon oxide matrix.

More precisely, the said polyoxometalates present within the said matrix are trapped in the walls of the said matrix. The said polyoxometalates are therefore not simply deposited, for

example by impregnation at the surface of the pores of the said matrix, but are located actually within the wall of the said matrix.

The characteristic localisation of the said polyoxometalates actually within the wall of the said mesostructured silicon oxide matrix enables a better interaction between the said matrix serving as a support and the active phase and/or its oxide precursors comprising the said polyoxometalates. This also results in improved retention of the textural and structural properties of the mesostructured silicon oxide matrices, improved maintenance of the structure of the said polyoxometalate and preferably of the said heteropolyanion following post-treatment of the final solid, as well as improved dispersion, heat resistance and chemical resistance of the said polyoxometalate.

In a terminological idiosyncrasy, and throughout the remainder of the text, polyoxometalates used according to the invention are herein defined as being the compounds corresponding to the formula  $(H_xX_xM_mO_y)^{q-}$ , wherein X is an element selected from phosphorus (P), silicon (Si), boron (B), nickel (Ni) and cobalt (Co), the said element being taken alone, M is one or more element(s) selected from molybdenum (Mo), tungsten (W), nickel (Ni) and cobalt (Co), O is oxygen, H is hydrogen, h is an integer within the range 0 to 12, x is an integer within the range 0 to 4, m is an integer equal to 5, 6, 7, 8, 9, 10, 11, 12 and 18, y is an integer within the range 17 to 72 and q is an integer within the range 1 to 20.

Preferably the element M cannot be a nickel atom or a cobalt atom alone.

The polyoxometalates defined according to the invention include two families of compounds, the isopolyanions and the heteropolyanions. These two compound families are defined in the article Heteropoly and Isopoly Oxometallates, Pope, Ed Springer-Verlag, 1983.

The isopolyanions which may be used in the present invention are polyoxometalates of the general formula  $(H_xX_xM_mO_y)^{q-}$ , wherein x=0, the other elements having the meaning given above.

Preferably, the m atoms of M of the said isopolyanions are either uniquely atoms of molybdenum, or uniquely atoms of tungsten, or a mixture of molybdenum and cobalt atoms, or a mixture of molybdenum and nickel atoms, or a mixture of tungsten and cobalt atoms, or a mixture of tungsten and nickel atoms. Among the m atoms of M of the said isopolyanions, the group VIII elements are partially substituted for the group VIB elements.

In particular, in the case wherein the m atoms of M are either a mixture of molybdenum atoms and cobalt atoms, or a mixture of molybdenum and nickel, or a mixture of tungsten and cobalt atoms, or a mixture of tungsten and nickel atoms, the cobalt and nickel atoms are partially substituted for the atoms of molybdenum and tungsten.

The m atoms of M of the said isopolyanions may similarly advantageously be either a mixture of nickel, molybdenum and tungsten atoms, or a mixture of cobalt, molybdenum and tungsten atoms.

In the case wherein the element M is molybdenum (Mo), m is preferably equal to 7. Similarly, in the case wherein the element M is tungsten (W), m is preferably equal to 12.

The isopolyanions (sic)  $Mo_7O_{24}^{6-}$  and  $H_2W_{12}O_{40}^{6-}$  are advantageously used as active phase precursors within the framework of the invention.

The said isopolyanions are advantageously formed by reaction of the oxoanions of type  $MO_4^{2-}$  with one another. For example, the molybdenum compounds are well known for this type of reaction since, according to the pH, the molybdenum compound in solution may be in the form  $MoO_4^{2-}$  or

in the form of an isopolyanion of the formula  $Mo_7O_{24}^{6-}$  which is obtained according to the reaction:  $7 MoO_4^{2-} + 8H^+ \rightarrow Mo_7O_{24}^{6-} + 4 H_2O$ . In the case of the isopolyanions in which M is a tungsten atom, the potential acidification of the reaction medium may, by provoking the formation of  $WO_4^{2-}$  tungstates, lead to the generation of  $\alpha$ -metatungstate, 12-fold condensed according to the following reaction:  $12 WO_4^{2-} + 18H^+ \rightarrow H_2W_{12}O_{40}^{6-} + 8H_2O$ .

The heteropolyanions which may be used in the present invention are polyoxometalates of the formula  $(H_xX_xM_mO_y)^{q-}$ , wherein x=1, 2, 3 or 4, the other elements having the meaning given above.

The heteropolyanions generally have a structure in which the element X is the "central" atom and the element M is a metal atom practically systematically in octahedral coordination, with  $X \neq M$ .

Preferably, the m atoms of M are either uniquely atoms of molybdenum, or uniquely atoms of tungsten, or a mixture of molybdenum and cobalt atoms, or a mixture of molybdenum and nickel, or a mixture of tungsten and molybdenum atoms, or a mixture of tungsten and cobalt atoms, or a mixture of tungsten and nickel atoms. The m atoms of M are preferably either uniquely atoms of molybdenum, or a mixture of atoms of molybdenum and cobalt, or a mixture of molybdenum and nickel. Preferably, the m atoms of M cannot be uniquely atoms of nickel, nor uniquely atoms of cobalt.

Among the m atoms of M of the said heteropolyanions, the group VIII elements are partially substituted for the group VIB elements.

In particular, in the case wherein the m atoms of M are either a mixture of molybdenum and cobalt atoms, or a mixture of molybdenum and nickel, or a mixture of tungsten and cobalt atoms, or a mixture of tungsten and nickel atoms, the cobalt and nickel atoms are partially substituted for the atoms of molybdenum and tungsten and preferably for the atoms of molybdenum.

The element X is preferably at least one atom of phosphorus.

The heteropolyanions are advantageously obtained by polycondensation of oxoanions of the type  $MO_4^{2-}$  around one or more oxoanion(s) of the type  $XO_4^{q-}$ , wherein the charge q is dictated by the octet rule and the position of the element X in the periodic table. There is then elimination of molecules of water and creation of oxo bridges between the atoms. These condensation reactions are governed by different experimental factors such as the pH, the concentration of the species in solution, the nature of the solvent, and the ratio m/x, being the ratio of the number of atoms of element M to the number of atoms of element X.

The heteropolyanions are negatively charged polyoxometalate species. To compensate for these negative charges, it is necessary to introduce counterions, and more particularly cations. These cations may advantageously be  $H^+$  protons, or any other cation of type  $NH_4^+$  or metal cations and, in particular, metal cations of the group VIII metals.

In the case where the counterions are protons, the molecular structure comprising the heteropolyanion and at least one proton constitutes a heteropolyacid. The heteropolyacids which may be used as active phase precursors in the present invention may be, by way of example, phosphomolybdic acid ( $3H^+, PMo_{12}O_{40}^{3-}$ ), or the acid phosphotungstate ( $3H^+, PW_{12}O_{40}^{3-}$ ).

In the case where the counterions are not protons, the term heteropolyanion salt is then used to designate this molecular structure. The association within the same molecular structure may then be advantageously exploited, via the use of a heteropolyanion salt, of the metal M and its promoter,

that is to say the element cobalt and/or the element nickel which may either be in position X within the structure of the heteropolyanion, or in partial substitution for at least one atom M of molybdenum and/or of tungsten within the structure of the heteropolyanion, or in counterion position.

Preferably, the polyoxometalates used according to the invention are the compounds corresponding to the formula  $(H_hX_xM_mO_y)^{q-}$ , wherein X is an element selected from phosphorus (P), silicon (Si), boron (B), nickel (Ni) and cobalt (Co), the said element being taken alone, M is one or more element(s) selected from molybdenum (Mo), tungsten (W), nickel (Ni) and cobalt (Co), O is oxygen, H is hydrogen, h is an integer within the range 0 to 6, x is an integer which may be equal to 0, 1 or 2, m is an integer equal to 5, 6, 7, 9, 10, 11 or 12, y is an integer within the range 17 to 48 and q is an integer within the range 3 to 12.

More preferably, the polyoxometalates used according to the invention are the compounds corresponding to the formula  $(H_hX_xM_mO_y)^{q-}$ , wherein h is an integer equal to 0, 1, 4 or 6, x is an integer equal to 0, 1 or 2, m is an integer equal to 5, 6, 10 or 12, y is an integer equal to 23, 24, 38, or 40, and q is an integer equal to 3, 4, 6 and [sic] 7, X, M, H and O having the meaning given above.

The preferred polyoxometalates used according to the invention are advantageously selected from the polyoxometalates of the formula  $PMo_{12}O_{40}^{3-}$ ,  $HPCoMo_{11}O_{40}^{6-}$ ,  $HPNiMo_{11}O_{40}^{6-}$ ,  $P_2Mo_5O_{23}^{6-}$ ,  $Co_2MO_{10}O_{38}H_4^{6-}$ ,  $CoMo_6O_{24}H_6^{3-}$  taken alone or in admixture.

Preferred polyoxometalates which may be advantageously used as active phase precursors of the catalyst implemented in the process according to the invention are the heteropolyanions called Anderson heteropolyanions of general formula  $XM_6O_{24}^{q-}$  for which the ratio m/x is equal to 6 and wherein the elements X and M and the charge q have the meaning given above. The elements [sic] X is thus an element selected from phosphorus (P), silicon (Si), boron (B), nickel (Ni) and cobalt (Co), the said element being taken alone, M is one or more element(s) selected from molybdenum (Mo), tungsten (W), nickel (Ni) and cobalt (Co), and q is an integer within the range 1 to 20 and preferably within the range 3 to 12.

The specific structure of the said Anderson heteropolyanions is described in the article in *Nature*, 1937, 150, 850. The structure of the said Anderson heteropolyanions comprises 7 octahedrons positioned within the same plane and interconnected at the edges: out of the 7 octahedrons, 6 octahedrons surround the central octahedron containing the element X.

The Anderson heteropolyanions containing within their structure cobalt and molybdenum, or nickel and molybdenum are preferred. The Anderson heteropolyanions of the formula  $CoMo_6O_{24}H_6^{3-}$  and  $NiMo_6O_{24}H_6^{4-}$  are especially preferred. In conformity with the formula, in these Anderson heteropolyanions, the atoms of cobalt and nickel are respectively the heteroelements X of the structure.

Indeed, the said heteropolyanions combine, in the same structure, molybdenum and cobalt or molybdenum and nickel. In particular, when they are in the form of cobalt salts or nickel salt, these enable an atomic ratio of the said promoter to the metal M, and in particular an atomic ratio (Co and/or Ni)/Mo, within the range 0.4 to 0.6 to be achieved. This ratio of the said promoter (Co and/or Ni)/Mo within the range 0.4 to 0.6 is especially preferred for maximising the performance of these catalysts of hydrotreatment and in particular of hydrodesulphuration implemented in the process according to the invention.

In the case wherein the Anderson heteropolyanion contains cobalt and molybdenum within its structure, a mixture of the two monomeric forms of the formula  $CoMo_6O_{24}H_6^{3-}$  and

dimeric forms of the formula  $Co_2Mo_{10}O_{38}H_4^{6-}$  of the said heteropolyanion, the two forms being in equilibrium, may be advantageously used. In the case wherein the Anderson heteropolyanion contains cobalt and molybdenum within its structure, the said Anderson heteropolyanion is preferably dimeric of the formula  $Co_2Mo_{10}O_{38}H_4^{6-}$ .

In the case wherein the Anderson heteropolyanion contains nickel and molybdenum within its structure, a mixture of the two monomeric forms of the formula  $NiMo_6O_{24}H_6^{4-}$  and dimeric forms of the formula  $Ni_2Mo_{10}O_{38}H_4^{8-}$  of the said heteropolyanion, the two forms being in equilibrium, may be advantageously used. In the case wherein the Anderson heteropolyanion contains nickel and molybdenum within its structure, the said Anderson heteropolyanion is preferably monomeric of the formula  $NiMo_6O_{24}H_6^{4-}$ .

Salts of Anderson heteropolyanions may similarly be advantageously used as active phase precursors according to the invention. The said Anderson heteropolyanion salts are advantageously selected from the cobalt or nickel salts of the 6-molybdochalcobaltate monomeric ion, respectively of the formula  $CoMo_6O_{24}H_6^{3-}$ ,  $3/2CO^{2+}$  or  $CoMo_6O_{24}H_6^{3-}$ ,  $3/2Ni^{2+}$  having an atomic ratio of the said promoter (Co and/or Ni)/Mo of 0.41, the cobalt or nickel salts of the decamolybdochalcobaltate dimeric ion of the formula  $Co_2MO_{10}O_{38}H_4^{6-}$ ,  $3Co^{2+}$  or  $Co_2Mo_{10}O_{38}H_4^{6-}$ ,  $3Ni^{2+}$  having an atomic ratio of the said promoter (Co and/or Ni)/Mo of 0.5, the cobalt or nickel salts of the 6-molybdonickellate ion of the formula  $NiMo_6O_{24}H_6^{4-}$ ,  $2Co^{2+}$  or  $NiMo_6O_{24}H_6^{4-}$ ,  $2Ni^{2+}$  having an atomic ratio of the said promoter (Co and/or Ni)/Mo of 0.5, and the cobalt or nickel salts of the decamolybdonickellate dimeric ion of the formula  $Ni_2Mo_{10}O_{38}H_4^{8-}$ ,  $4Co^{2+}$  or  $Ni_2Mo_{10}O_{38}H_4^{8-}$ ,  $4Ni^{2+}$  having an atomic ratio of the said promoter (Co and/or Ni)/Mo of 0.6.

The Anderson heteropolyanion salts highly preferably used in the invention are selected from the salts of dimeric heteropolyanions including cobalt and molybdenum within their structure of the formula  $Co_2Mo_{10}O_{38}H_4^{6-}$ ,  $3Co^{2+}$  and  $Co_2Mo_{10}O_{38}H_4^{6-}$ ,  $3Ni^{2+}$ . A salt of Anderson heteropolyanions that is yet more preferred is the salt of dimeric Anderson heteropolyanion of the formula  $Co_2Mo_{10}O_{38}H_4^{6-}$ ,  $3Co^{2+}$ .

Other preferred polyoxometalates which may be advantageously used as active phase precursors of the catalyst implemented in the process according to the invention are the Keggin heteropolyanions of general formula  $XM_{12}O_{40}^{q-}$  for which the m/x ratio is equal to 12, and the lacunary Keggin heteropolyanions of general formula  $XM_{11}O_{39}^{q-}$  for which the m/x ratio is equal to 11 and wherein the elements X and M and the charge q have the meanings given above. X is thus an element selected from phosphorus (P), silicon (Si), boron (B), nickel (Ni) and cobalt (Co), the said element being taken alone, M is one or more element(s) selected from molybdenum (Mo), tungsten (W), nickel (Ni) and cobalt (Co), and q is an integer within the range 1 to 20 and preferably 3 to 12.

The said Keggin species are advantageously obtained for variable pH ranges according to the pathways for obtaining them described in the publication of A. Griboval, P. Blanchard, E. Payen, M. Fournier, and J. L. Dubois, *Chem. Lett.*, 1997, 12, 1259.

A preferred Keggin type heteropolyanion that is advantageously used as an active phase precursor according to the invention, is the heteropolyanion of the formula  $PMo_{12}O_{40}^{3-}$ .

The preferred Keggin heteropolyanion may also be advantageously used in the invention in its heteropolyacid form of the formula  $PMo_{12}O_{40}^{3-}$ ,  $3H^+$ .

In the said Keggin type heteropolyanions of the above formula, at least one atom of molybdenum is substituted with a nickel atom, a cobalt atom, or with at least one atom of vanadium respectively.

The said heteropolyanions mentioned above are described in the publications of L. G. A. van de Water, J. A. Bergwerff, Bob, G. Leliveld, B. M. Weckhuysen, and K. P. de Jong, *J. Phys. Chem. B*, 2005, 109, 14513 and de D. Soogund, P. Lecour, A. Daudin, B. Guichard, C. Legens, C. Lamonié, and E. Payen in *Appl. Catal. B*, 2010, 98, 1, 39.

Salts of Keggin or lacunary Keggin type heteropolyanions may similarly be advantageously used as active phase precursors according to the invention. Salts of preferred Keggin or lacunary Keggin type heteropolyanion or heteropolyacids are advantageously selected from the cobalt or nickel salts of phosphomolybdc, siliconmolybdc, phosphotungstic or silicotungstic acids. The said salts of Keggin or lacunary Keggin type heteropolyanion or heteropolyacids are described in U.S. Pat. No. 2,547,380. Preferably, a Keggin type heteropolyanion salt is nickel phosphotungstate of the formula  $3/2\text{Ni}^{2+}\text{PW}_{12}\text{O}_{40}^{3-}$  having an atomic ratio of the group VI metal to the group VIII metal, that is Ni/W, of 0.125.

Other salts of Keggin or lacunary Keggin type heteropolyanions or heteropolyacids that may be advantageously used as active phase precursors according to the invention are the heteropolyanion or heteropolyacid salts of general formula  $Z_x\text{XM}_{12}\text{O}_{40}$  (or  $xZ^{p+}\text{XM}_{12}\text{O}_{40}^{p-x-}$ , formula manifesting the counterion  $Z^{p+}$ ), wherein Z is cobalt and/or nickel, X is phosphorus, silicon or boron and M is molybdenum and/or tungsten, x takes the value of 2 or more if X is phosphorus, of 2.5 or more if X is silicon and of 3 or more if X is boron. Such salts of Keggin or lacunary Keggin type heteropolyanions or heteropolyacids are described in French Patent 2749778. These structures offer the particular benefit as compared with the structures described in U.S. Pat. No. 2,547,380 of achieving higher atomic ratios of the group VIII element to the element of group VI, in particular higher than 0.125.

This increase in the said ratio is obtained by reducing the said salts of Keggin or lacunary Keggin type heteropolyanion or heteropolyacids salts. Thus the presence of at least part of the molybdenum and/or of the tungsten is at a lower valence than its normal value of six such as results, for example, from the composition of phosphomolybdc, phosphotungstic, siliconmolybdc or silicotungstic acid.

Higher atomic ratios of the group VIII element to the element of group VI are especially preferred to maximise the performances of the hydrotreatment catalysts and in particular of the hydrodesulphuration catalysts implemented in the process according to the invention.

The salts of Keggin type substituted heteropolyanions of the formula  $Z_x\text{XM}_{11}\text{O}_{40}Z'\text{C}_{(z-2-x)}$ , wherein Z' is substituted for an M atom and wherein Z is cobalt and/or nickel, X is phosphorus, silicon or boron and M is molybdenum and/or tungsten, Z' is cobalt, iron, nickel, copper or zinc, and C is an  $\text{H}^+$  ion or an alkylammonium cation, x takes the value of 0 to 4.5, z a value between 7 and 9; the said salts being described in French Patent 2764211 may similarly be advantageously used as active phase precursors according to the invention.

Thus, the said salts of Keggin heteropolyanions correspond to those described in French Patent 2749778 but in which a Z' atom is substituted for an atom M. The said salts of substituted Keggin heteropolyanions are especially preferred because they lead to atomic ratios between the group VIII element and that of group VI of up to 0.5.

The nickel salts of a lacunary Keggin type heteropolyanion described in French patent application FR2935139 may similarly be advantageously used as active phase precursors

according to the invention. The nickel salts of a lacunary Keggin type heteropolyanion comprising tungsten in its structure are of the general formula  $\text{Ni}_{x+y/2}\text{XW}_{11-y}\text{O}_{39-5/2z}\text{zH}_2\text{O}$ , wherein Ni is nickel, X is selected from phosphorus, silicon and boron, W is tungsten, O is oxygen,  $y=0$  or  $2$ ,  $x=3.5$  if X is phosphorus,  $x=4$  if X is silicon,  $x=4.5$  if X is boron and z is a number within the range 0 to 36, and wherein the said molecular structure does not have a nickel atom in substitution for a tungsten atom in its structure, the 10 said nickel atoms being in a counterion position in the structure of the said compound. An advantage of this invention is given by the increased solubility of these heteropolyanion salts.

Other preferred polyoxometalates which may be advantageously used as active phase precursors of the catalyst implemented in the process according to the invention are the Strandberg heteropolyanions of the formula  $\text{H}_h\text{P}_2\text{Mo}_5\text{O}_{23}^{(6-h)-}$ , wherein h is equal to 0, 1 or 2 and for which the m/x ratio is equal to 5/2.

20 The preparation of the said Strandberg heteropolyanions is described in the article by de W-C. Cheng, N. P. Luthra, *J. Catal.*, 1988, 109, 163. This has been demonstrated by J. A. Bergwerff, T. Visser, B. R. G. Leliveld, B. D. Rossenaar, K. P. de Jong, and B. M. Weckhuysen, *Journal of the American Chemical Society* 2004, 126, 44, 14548.

An especially preferred Strandberg heteropolyanions [sic] used in the invention is the heteropolyanion of the formula  $\text{P}_2\text{Mo}_5\text{O}_{23}^6$ .

Thus, through the use of different methods of preparation, 30 numerous polyoxometalates and their associated salts are available, with variable promoter X/metal M ratios. Generally, all these polyoxometalates and their associated salts may be advantageously used for the preparation of the catalysts implemented in the process according to the invention. However, the above list is not exhaustive, and other combinations may be envisaged.

The use of polyoxometalates for the preparation of a catalyst implemented in the process according to the invention has numerous catalytic advantages. The said polyoxometalates which are oxide precursors combining within the same molecular structure at least one group VIB element, preferably molybdenum and/or tungsten and/or at least one group VIII element, preferably cobalt and/or nickel, give rise, following sulphuration, to catalysts the catalytic performances 45 of which are improved due to a better promotion effect, that is, a better synergy between the group VIB element and the group VIII element.

The catalyst implemented in the process according to the invention preferably comprises a content of the group VIB element by mass, expressed as wt. % of oxide relative to the total mass of the catalyst, within the range 1 to 30 wt. %, preferably within the range 5 to 25 wt. % and preferably within the range 8 to 23 wt. %.

The said contents are the total contents of group VIB element whatever the form of the said group VIB element present in the said catalyst and optionally whatever its mode of introduction. The said contents are thus representative of the content of group VIB element present either in the form of at least one polyoxometalate within the mesostructured silicon oxide matrix, or in any other form depending on its mode of introduction, such as for example in the oxide form.

Preferably, the catalyst implemented in the process according to the invention comprises a content by mass of the group VIII element expressed in percentage by weight of oxide relative to the total mass of the catalyst within the range 0.1 to 10 wt. %, preferably within the range 1 to 7 wt. % and preferably within the range 2 to 6 wt. %.

## 11

The said contents are the total contents of group VIII elements whatever the form of the said group VIII element present in the said catalyst and as applicable whatever its mode of introduction. The said contents are thus representative of the content of group VIII element present either in the form of at least one polyoxometalate within the mesostructured silicon oxide matrix whether in position M or in position X, or present in counterion form and/or optionally added at different stages in the preparation of the said mesostructured silicon oxide matrix as described below, or in any other form depending on its mode of introduction, such as for example in the oxide form.

Preferably, the catalyst implemented in the process according to the invention comprises a content by mass of doping element X selected from phosphorus, boron and silicon within the range 0.1 to 10 wt. %, preferably 1 to 6 wt. %, and yet more preferably 2 to 5 wt. % of oxide relative to the final catalyst.

The said contents are the total contents of doping elements selected from phosphorus, boron and silicon whatever the form of the said doping element present in the said catalyst and whatever its mode of introduction. The said contents are thus representative both of the content of the doping element selected from phosphorus, boron and silicon present in the form of at least one polyoxometalate within the mesostructured silicon oxide matrix in position X and/or optionally added at different stages in the preparation of the said mesostructured silicon oxide matrix as described below, or in any other form depending on its mode of introduction, such as for example in the oxide form.

According to the invention, the said polyoxometalates defined above are present within a mesostructured silicon oxide matrix having a pore size within the range 1.5 to 50 nm and having amorphous walls of thickness within the range 1 to 30 nm and preferably 1 to 10 nm.

Mesostructured oxide matrix is understood within the meaning of the present invention as an inorganic solid having a porosity organised on the scale of the mesopores of each of the elementary particles constituting the said solid, that is, a porosity organised on the scale of pores of uniform size within the range 1.5 to 50 nm and preferably 1.5 to 30 nm and yet more preferably 4 to 16 nm, and homogeneously and regularly distributed within each of the said particles constituting the matrix. The matter located between the mesopores of each of the elementary particles of the oxide matrix of the precursor of the catalyst used in the process according to the invention is amorphous and forms sides or walls, the thickness of which is within the range 1 to 30 nm and preferably 1 to 10 nm. The thickness of the walls corresponds to the distance separating one pore from another. The organisation of the mesoporosity described above leads to a structuring of the oxide matrix which may be hexagonal, vermicular or cubic and preferably hexagonal.

Generally, the said "mesostructured" materials are advantageously obtained by methods of synthesis called "soft chemistry" (G. J. de A. A. Soler-Illia, C. Sanchez, B. Lebeau and J. Patarin, Chem. Rev., 2002, 102, 4093) at low temperatures via la coexistence, in aqueous solution or in highly polar solvents, of inorganic precursors and structuring agents, generally ionic or neutral molecular or supramolecular surfactants. Control of the electrostatic interactions or by hydrogen bonds between the inorganic precursors and the structuring agent conjointly linked to hydrolyse/condensation reactions of the inorganic precursor leads to a cooperative assembly of the organic and inorganic phases generating micellar aggregates of surfactants of uniform size that is controlled within an inorganic matrix. This phenomenon of cooperative auto-

## 12

assembly governed, *inter alia*, by the concentration of structuring agent may be induced by gradual evaporation of a solution of reactants the structuring-agent concentration of which is lower than the critical micellar concentration, or else via the precipitation or direct gelification of the solid when using a solution of precursors that has a higher reactant concentration.

Freeing of the porosity is then achieved by eliminating the surfactant, this being done conventionally by methods of chemical extraction, or by heat treatment.

A number of families of mesostructured materials have been developed, as a function of the nature of the inorganic precursors and of the structuring agent used, as well as of the operating conditions imposed. The M41S family consists of mesoporous materials obtained by the use of ionic surfactants such as quaternary ammonium salts having a generally hexagonal, cubic or lamellar structure, pores of uniform size within a range of 1.5 to 10 nm and amorphous walls of thickness of the order of 1 to 2 nm. The M41S family was initially developed by Mobil in the article by J. S. Beck, J. C. Vartuli, W. J. Roth, M. E. Leonowicz, C. T. Kresge, K. D. Schmitt, C. T.-W. Chu, D. H. Olson, E. W. Sheppard, S. B. McCullen, J. B. Higgins, and J. L. Schlenker, J. Am. Chem. Soc., 1992, 114, 27, 10834.

The family of materials known by the name SBA is characterised by the use of amphiphilic macromolecular structuring agents of the block copolymer type. These materials are characterised by a generally hexagonal, cubic or lamellar structure, pores of uniform size within a range of 4 to 50 nm and amorphous walls of thickness within a range of 3 to 7 nm.

The mesostructured oxide matrix used in the catalyst implemented in the process according to the invention is purely silica.

The mesostructured silicon oxide matrix used in the catalyst implemented in the process according to the invention is advantageously a mesostructured matrix belonging to the M41S family or to the SBA family of materials.

Preferably, the said mesostructured silicon oxide matrix is a matrix of the type SBA-15.

According to the invention, the said polyoxometalates defined above are present within a mesostructured silicon oxide matrix. More precisely, the said polyoxometalates present within the said mesostructured silicon oxide matrix are trapped actually within the said matrix.

Preferably, the said polyoxometalates are present in the walls of the said mesostructured matrix. Occlusion of the said polyoxometalates in the walls of the said mesostructured matrix is achievable by a method of synthesis termed direct, at the time of synthesis of the said matrix serving as a support by addition of desired polyoxometalates to the precursor reactants of the inorganic oxide lattice of the matrix.

The said mesostructured silicon oxide matrix comprising the said polyoxometalates trapped in its walls implemented in the process according to the invention is advantageously prepared exclusively by direct synthesis.

More precisely, the said mesostructured silicon oxide matrix is advantageously obtained according to a method of preparation comprising: a) a step of formation of at least one polyoxometalate of the formula given above according to a method known to the person skilled in the art, b) a step of mixing in solution at least one surfactant, at least one silica precursor, then at least one polyoxometalate obtained according to step a) to obtain a colloidal solution, c) a step of maturation of the said colloidal solution obtained at the end of step b) in time and in temperature d) an optional step of autoclaving of the suspension obtained at the end of step c), e) a step of filtration of the suspension obtained at the end of step

c) and following optional passage into the autoclaving step, of washing and drying of the solid thus obtained, f) a step of eliminating the said surfactant leading to generation of the uniform and organised mesoporosity of the mesostructured matrix, g) an optional step of treatment of the solid obtained at the end of step f) in order to partially or wholly regenerate the polyoxometalate entity that may have been partially or totally degraded during step f) and h) a step of optional drying of the said solid thus obtained consisting of the said mesostructured silicon oxide matrix comprising the said polyoxometalates trapped in its walls.

Step a) of formation of at least one polyoxometalate of the formula given above is advantageously implemented according to a method known to the person skilled in the art. Preferably, the polyoxometalates described above, and their associated methods of preparation are used in the method of preparation of the said mesostructured silicon oxide matrix comprising the said polyoxometalates trapped in its walls.

Step b) of the said method of preparation consists in mixing, in solution, at least one surfactant and at least one silica precursor, then at least one polyoxometalate obtained according to step a) to obtain a colloidal solution.

Preferably, at least one surfactant and at least one silica precursor are mixed in solution for a duration within the range 15 minutes to 1 hour, then at least one polyoxometalate obtained according to step a) in admixture in a solution of the same nature and preferably the same solution is added to the previous solution to obtain a colloidal solution.

Mixing step b) is performed with agitation at a temperature within the range 25° C. to 30° C. and preferably within the range 25° C. to 50° C. for a duration within the range 5 minutes to 2 h and preferably 30 minutes to 1 h.

The solution in which are mixed at least one surfactant, at least one polyoxometalate obtained according to step a) and at least one silica precursor conforming to step b) of the said method of preparation may advantageously be acidic, basic or neutral. Preferably, the said solution is acidic or neutral. The acids used to obtain an acidic solution are advantageously selected from hydrochloric acid, sulphuric acid and nitric acid. The said solution may advantageously be aqueous or may advantageously be a mixture of water and organic solvent, the organic solvent preferably being a polar solvent, preferably an alcohol, and more preferably, the solvent is ethanol. The said solution may also be advantageously practically organic, preferably practically alcoholic, the quantity of water being such that the hydrolysis of the inorganic precursors is assured. The quantity of water is thus preferably stoichiometric. Very preferably, the said solution is an acidic aqueous solution.

The surfactant used for preparing the mixture in step b) of the said method of preparation is an ionic or non-ionic surfactant, or a mixture of the two. Preferably, the ionic surfactant is selected from the ions phosphonium and ammonium and highly preferentially from the quaternary ammonium salts such as cetyltrimethylammonium bromide (CTAB). Preferably, the non-ionic surfactant may be any copolymer having at least two parts of differing polarities conferring upon them amphiphilic macromolecular properties. These copolymers may comprise at least one block forming part of the non-exhaustive list of families of the following polymers: the fluorinated polymers (—[CH<sub>2</sub>—CH<sub>2</sub>—CH<sub>2</sub>—CH<sub>2</sub>—O—CO—R1- where R1=C<sub>4</sub>F<sub>9</sub>, C<sub>8</sub>F<sub>17</sub>, etc.], the biological polymers such as the amino polyacids (poly-lysine, alginates, etc.), the dendrimers, the polymers consisting of chains of poly(alkylene oxide). In general, any copolymer of amphiphilic character known to the person skilled in the art may be used (S. Förster and M. Antionnetti, *Adv. Mater.*, 1998,

10, 195; S. Förster and T. Plantenberg, *Angew. Chem. Int. Ed.*, 2002, 41, 688; H. Cölfen, *Macromol. Rapid Commun.*, 2001, 22, 219). Preferably, a block copolymer consisting of chains of poly(alkylene oxide) is used. The said block copolymer is preferably a block copolymer having two, three or four blocks, each block consisting of a poly(alkylene oxide) chain. For a two-block copolymer, one of the blocks consists of a poly(alkylene oxide) chain of a hydrophilic nature and the other block consists of a poly(alkylene oxide) chain of a hydrophobic nature. For a three-block copolymer, at least one of the blocks consists of a poly(alkylene oxide) chain of a hydrophilic nature, while the other at least one block consists of a poly(alkylene oxide) chain of a hydrophobic nature. Preferably, in the case of a three-block copolymer, the poly(alkylene oxide) chains of a hydrophilic nature are poly(ethylene oxide) chains denoted (PEO)<sub>x</sub> and (PEO)<sub>z</sub>, and the poly(alkylene oxide) chains of a hydrophobic nature are poly(propylene oxide) chains denoted (PPO)<sub>y</sub>, poly(butylene oxide) chains, or mixed chains each of which is a mixture of a plurality of monomers of alkylene oxide. In the case of a three-block copolymer, a compound of the formula (PEO)<sub>x</sub>-(PPO)<sub>y</sub>-(PEO)<sub>z</sub>, is highly preferably used, wherein x is within the range 5 to 300 and y is within the range 33 to 300 and z is within the range 5 to 300. Preferably, the values of x and z are identical. Highly advantageously, a compound wherein x=20, y=70 and z=20 (P123) and a compound wherein x=106, y=70 and z=106 (F127) are used. The commercial non-ionic surfactants known by the names Pluronic (BASF), Tetronic (BASF), Triton (Sigma), Tergitol (Union Carbide), and Brij (Aldrich) are usable as non-ionic surfactants. For a four-block copolymer, two of the blocks consist of a poly(alkylene oxide) chain of a hydrophilic nature and the other two blocks consist of a poly(alkylene oxide) chain of a hydrophobic nature. Preferably, for preparing the mixture of step b) of the said method of preparation, the mixture of an ionic surfactant such as CTAB and a non-ionic surfactant such as P123 are preferably used.

As the mesostructured oxide matrix used in the catalyst implemented in the process according to the invention is purely silica, the silica precursor(s) used to form the mesostructured oxide matrix is(are) obtained from any source of silica and advantageously from a sodium silicate precursor of the formula Na<sub>2</sub>SiO<sub>3</sub>, a chlorinated precursor of the formula SiCl<sub>4</sub>, an alkoxide precursor of the formula Si(OR)<sub>4</sub> wherein R=H, methyl or ethyl, or a chloroalkoxide precursor of the formula Si(OR)<sub>4-x</sub>Cl<sub>x</sub> wherein R=H, methyl or ethyl, x being within the range 0 to 4. The silica precursor may also advantageously be an alkoxide precursor of the formula Si(OR)<sub>4-x</sub>R'<sub>x</sub> wherein R=H, methyl or ethyl and R' is an alkyl chain or an alkyl chain functionalised, for example, with a thiol, amino, β-diketone or sulphonic acid group, x being within the range 0 to 4.

A preferred silica precursor is tetraethylorthosilicate (TEOS) of the formula Si(OEt)<sub>4</sub>.

The polyoxometalates described above and having the general formula previously mentioned are used in step b) of the method of preparing the said mesostructured silicon oxide matrix comprising the said polyoxometalates trapped in its walls.

The preferred polyoxometalates selected from the Anderson heteropolyanion salts of dimeric type containing within their structure cobalt and molybdenum preferably of the formula Co<sub>2</sub>Mo<sub>10</sub>O<sub>38</sub>H<sub>4</sub><sup>6-</sup>, 3Co<sup>2+</sup> and Co<sub>2</sub>Mo<sub>10</sub>O<sub>38</sub>H<sub>4</sub><sup>6-</sup>, 3Ni<sup>2+</sup>, the Keggin heteropolyanion of the formula PMo<sub>12</sub>O<sub>40</sub><sup>3-</sup> and the Strandberg heteropolyanion of the formula P<sub>2</sub>Mo<sub>5</sub>O<sub>23</sub><sup>6-</sup>.

## 15

Step c) of the said method of preparation consists in a maturation step, that is, a step of conservation, under agitation, of the said colloidal solution obtained at the end of step b) at a temperature within the range 25° C. to 80° C. and preferably within the range 25° C. to 40° C. for a duration within the range 1 h to 48 h and preferably 20 h to 30 h.

At the end of maturation step c), a suspension is obtained.

The optional step d) of the said preparation method consists in optionally autoclaving the suspension obtained at the end of step c). This step consists in placing the said suspension in a sealed chamber at a temperature within the range 80° C. to 140° C., preferably within the range 90° C. to 120° C. and more preferentially within the range 100° C. to 110° C. so as to work at autogenic pressure inherent to the operating conditions selected. The autoclaving is maintained for a duration within the range 12 to 48 hours and preferably 15 to 30 hours.

The suspension obtained at the end of step c) is then filtered according to step e) and the solid thus obtained is washed and dried. The washing of the said solid obtained after filtration and before drying is advantageously carried out with a solution of the same nature as the solution wherein are mixed at least one surfactant, at least one heteropolyanion and at least one silica precursor in conformity with step b) of the said preparation method, then with an aqueous solution of distilled water.

The drying of the said solid obtained after filtration and washing in the course of step e) of the said method of preparation is advantageously carried out in an oven at a temperature within the range 25° C. to 140° C., preferably 25° C. to 100° C. and preferably 30° C. to 80° C. during a period within the range 10 to 48 h and preferably within the range 10 to 24 h.

Step f) then consists of a step of elimination of the said surfactant, leading to the generation of the uniform and organised mesoporosity of the mesostructured matrix.

The elimination of the surfactant in the course of step f) of the said method of preparation in order to obtain the mesostructured matrix used according to the invention is advantageously performed by heat treatment, and preferably by calcination in air at a temperature within the range 300° C. to 1000° C. and preferably at a temperature within the range 400° C. to 600° C. during a period within the range 1 to 24 hours and preferably during a period within the range 6 to 20 hours.

Step f) is optionally followed by step g) of treatment of the solid in order to regenerate at least partially or wholly the polyoxometalate entity that may have been at least partially or totally degraded in step f). In the case of the said polyoxometalate being totally degraded in step f), the said regeneration step g) is obligatory. This step advantageously consists in washing of the solid with a polar solvent while using a Soxhlet type extractor. Preferably, the extraction solvent is selected from the alcohols, acetonitrile and water. Preferably the solvent is an alcohol and highly preferably the solvent is methanol. The said washing is carried out during a period within the range 1 to 24 hours, and preferably 1 to 8 hours at a temperature within the range 65 to 110° C. and preferably within the range 90 to 100° C.

Extraction with the polar solvent makes it possible not only to reform the said polyoxometalates trapped in the walls of the said matrix but also to eliminate the said polyoxometalates that may have formed at the surface of the said matrix.

In the case wherein step g) is obligatory, the said step g) is followed by step h). Step h) consists in a step of drying of the said solid thus obtained, the said solid consisting of the said mesostructured silicon oxide matrix comprising the said

## 16

polyoxometalates trapped in its walls. The drying of the said solid is advantageously performed in an oven or in a drying cupboard at a temperature within the range 40° C. to 140° C. preferably 40° C. to 100° C. and for a duration within the range 10 to 48 h and preferably 10 to 24 h.

The said mesostructured silicon oxide matrix comprising the said polyoxometalates trapped in its walls that is implemented in the process according to the invention advantageously has a specific surface area within the range 100 to 1000 m<sup>2</sup>/g and highly advantageously within the range 300 to 500 m<sup>2</sup>/g.

The said mesostructured oxide matrix comprising the said polyoxometalates trapped in its walls, that is, the catalyst in its oxide form, exhibits a form of each of the elementary particles of which it is composed that is non-homogeneous, that is, an irregular and preferably non-spherical shape. The said elementary particles constituting the said matrix comprising the said polyoxometalates trapped in its walls are preferably non-spherical.

At the end of the method of preparation by direct synthesis, the said elementary particles constituting the said matrix comprising the said polyoxometalates trapped in its walls advantageously present a mean size within the range 50 nm to 10 microns and preferably within the range 50 nm to 1 micron.

Other elements may advantageously be added at different stages in the preparation of the said mesostructured silicon oxide matrix used in the invention. The said elements are preferably selected from the group VIII elements called promoters, the doping elements and the organic compounds. Highly preferably, the said group VIII metal is selected from nickel and cobalt and more preferably, the group VIII metal consists uniquely of cobalt or nickel. Still more preferably, the group VIII metal is cobalt. The doping elements are preferably selected from boron, silicon, phosphorus and fluorine.

The said elements may advantageously be added alone or in admixture in the course of one or more steps of the method of preparing the said matrix selected from steps i), ii), iii) and iv) below.

i) The said elements may advantageously be introduced during step b) of mixing in solution of at least one surfactant, of at least one silica precursor, then of at least one polyoxometalate obtained according to step a) to obtain a colloidal solution, of the method of preparing the said matrix.

ii) The said elements may advantageously be introduced after step f) and before step g) of the said preparation method. The said elements may advantageously [be] introduced by any technique known to the person skilled in the art and advantageously by dry impregnation.

iii) The said elements may be advantageously introduced after drying step h) of the said preparation method prior to forming. The said elements may advantageously be introduced by any technique known to the person skilled in the art and advantageously by dry impregnation.

iv) The said elements may advantageously be introduced after the step of forming of the said matrix. The said elements may advantageously be introduced by any technique known to the person skilled in the art and advantageously by dry impregnation.

After each of steps ii) iii) or iv) described above, the solid obtained consisting of the said mesostructured silicon oxide matrix comprising the said polyoxometalates trapped in its walls may advantageously undergo a drying step and optionally a step of calcination in optionally O<sub>2</sub>-enriched air at a temperature within the range 200 to 600° C. and preferably

within the range 300 to 500° C. for a duration within the range 1 to 12 hours and preferably for a duration within the range 2 to 6 hours.

The sources of group VIII elements that may advantageously be used are well known to the person skilled in the art. The nitrates preferably selected from cobalt nitrate and nickel nitrate, the sulphates, the hydroxides selected from the cobalt hydroxides and the nickel hydroxides, the phosphates, the halogenides selected from the chlorides, the bromides and the fluorides, the carboxylates selected from the acetates and the carbonates may advantageously be used as sources of group VIII elements.

The group VIII promoter elements are advantageously present in the catalyst in contents within the range 0.1 to 10 wt. %, preferably 1 to 7 wt. % of oxide with reference to the final catalyst.

The doping elements that may advantageously be introduced are advantageously selected from boron, silicon, phosphorus and fluorine taken alone or in admixture. The doping element is an added element which has no catalytic character per se, but which increases the catalytic activity of the metal(s).

The said doping element may be advantageously introduced alone or in admixture during the synthesis of the said material used in the invention. It may also be introduced by impregnation of the material used according to the invention before or after drying, before or after re-extraction. Finally, the said dopant may be introduced by impregnation of the said material used in the invention after forming.

The doping elements are advantageously present in the catalyst used according to the present invention in a content within the range 0.1 to 10 wt. %, preferably 0.5 to 8 wt. %, and yet more preferably 0.5 to 6 wt. % of oxide with reference to the final catalyst.

The source of boron may advantageously be boric acid, preferably orthoboric acid  $H_3BO_3$ , ammonium diborate or pentaborate, boric oxide, [and] the boric esters. Boron may also be introduced at the same time as the group VIB element(s) in the form of Keggin heteropolyanions, lacunary Keggin-type heteropolyanions, substituted Keggin heteropolyanions, such as, for example, in the form of boromolybdic acid and the salts thereof, or borotungstic acid and the salts thereof during the synthesis of the said matrix. Boron, when not introduced during the synthesis of the said matrix, but post-impregnation, may be advantageously introduced for example with a solution of boric acid in a water/alcohol mixture, or in a water/ethanolamine mixture. Boron may also be advantageously introduced in the form of a mixture of boric acid, oxygenated water and a basic organic compound containing nitrogen, such as ammonia, the primary and secondary amines, the cyclic amines, the compounds of the pyridine and quinoline family and the compounds of the pyrrole family.

The source of phosphorus may advantageously be orthophosphoric acid  $H_3PO_4$ , the corresponding salts and esters or the ammonium phosphates. Phosphorus may also be advantageously introduced at the same time as the group VIB element(s) in the form of Keggin heteropolyanions, lacunary Keggin-type heteropolyanions, substituted Keggin heteropolyanions, or Strandberg-type heteropolyanions such as, for example, in the form of phosphomolybdic acid and the salts thereof, or phosphotungstic acid and the salts thereof during the synthesis of the said matrix. Phosphorus, when not introduced during the synthesis of the said matrix, but post-impregnation, may be advantageously introduced in the form of a mixture of phosphoric acid and a basic organic compound containing nitrogen, such as ammonia, the primary and sec-

ondary amines, the cyclic amines, the compounds of the pyridine and quinoline family and the compounds of the pyrrole family.

The sources of fluorine that may be advantageously used are well known to the person skilled in the art. For example, the fluoride anions may be introduced in the form of hydrofluoric acid or the salts thereof. These salts are formed with alkali metals, ammonium or an organic compound. In the latter case, the salt is advantageously formed in the reaction mixture by reaction between the organic compound and the hydrofluoric acid. Fluorine, when not introduced during the synthesis of the said matrix, but post-impregnation, may be advantageously introduced for example by impregnation of an aqueous solution of hydrofluoric acid, or of ammonium fluoride or ammonium difluoride.

Once the doping element has been introduced post-impregnation, the person skilled in the art may advantageously proceed to drying at a temperature advantageously within the range 90 to 150° C. and for example at 120° C., and possibly thereafter to calcination preferably in air on a current-carrying bed, at a temperature advantageously within the range 300 to 700° C. and for example at 450° C. for 4 hours.

The added organic compounds are preferably selected from the chelating agents, the non-chelating agents, the reducing agents and the additives known to the person skilled in the art. The said organic compounds are advantageously selected from the optionally etherified mono-, di- or polyalcohols, the carboxylic acids, the sugars, the non-cyclic mono-, di- or polysaccharides such as glucose, fructose, maltose, lactose or sucrose, the esters, the ethers, the crown ethers, compounds containing sulphur or nitrogen, such as nitriloacetic acid, ethylenediaminetetraacetic acid, or diethylenetriamine.

The said mesostructured silicon oxide matrix comprising the said polyoxometalates trapped in its walls and serving as a support for the catalyst may be obtained in the form of powder, beads, pellets, granules or extrudates, the forming operations being performed according to the conventional techniques known to the person skilled in the art. Preferably, the said mesostructured silicon oxide matrix used according to the invention is obtained in powder form and used having been formed into extrudates or beads.

During these forming operations, it is also possible to add to the said mesostructured silicon oxide matrix comprising the said polyoxometalates trapped in its walls, at least one porous oxide material preferably selected from the group formed by alumina, silica, la silica-alumina, magnesium, clay, titanium oxide, zirconium oxide, lanthanum oxide, cerium oxide, the aluminium phosphates, the boron phosphates, or a mixture of at least two of the oxides mentioned above and the alumina-boron oxide combinations, the alumina-titanium mixtures, alumina-zirconia and titanium-zirconia. It is also possible to add the aluminates, such as for example the aluminates of magnesium, calcium, barium, manganese, iron, cobalt, nickel, copper and zinc, the mixed aluminates, such as for example those containing at least two of the metals mentioned above. It is also advantageously possible to add the titanates, such as for example the titanates of zinc, nickel and cobalt. It is also advantageously possible to use mixtures of alumina and silica and mixtures of alumina with other compounds such as, for example, the elements of group VIB, phosphorus, fluorine or boron. It is also possible to use simple synthetic or natural clays of the type 2:1 dioctahedral phyllosilicate or 3:1 trioctahedral phyllosilicate such as kaolinite, antigorite, chrysotile, montmorillonite, beidellite, vermiculite, talc, hectorite, saponite, laponite. These clays may optionally be delaminated. It is also advanta-

geously possible to use mixtures of alumina and clay and mixtures of silica-alumina and clay.

The said mesostructured silicon oxide matrix comprising the said polyoxometalates trapped in its walls is characterised by a plurality of analytical methods and notably by small-angle X-ray diffraction (small-angle XRD), wide-angle X-ray diffraction (XRD), nitrogen volumetry (BET), transmission electron microscopy (TEM) optionally linked to X-ray analysis, scanning electron microscopy (SEM), X-ray fluorescence (XRF) and by any technique known to the person skilled in the art for characterising the presence of polyoxometalates such as Raman spectroscopy in particular, and UV-visible or infra-red spectroscopy, as well as microanalyses. Methods such as nuclear magnetic resonance (NMR), or electron paramagnetic resonance (EPR) (notably with the use of reduced heteropolyanions) may also be used according to the type of heteropolyanions employed.

At the end of the preparation method described above, the catalyst presents, in its oxide form, in the form of a solid consisting of a mesostructured silicon oxide matrix comprising the said polyoxometalates trapped in its walls.

According to the invention, the said catalyst in its oxide form is sulphured before being implemented in the hydrodesulphuration process according to the invention.

This sulphuration step generates the sulphured active phase. Indeed, the transformation of at least one polyoxometalate trapped in the mesostructured oxide matrix in its associated sulphured active phase is advantageously achieved by sulphuration, that is, by a treatment at the temperature of the said matrix in contact with an organic sulphur compound that is degradable and generates  $H_2S$ , or directly in contact with a stream of  $H_2S$  diluted in  $H_2$  at a temperature within the range 200 to 600°C. and preferably within the range 300 to 500°C. according to methods well known to the person skilled in the art. More precisely, the sulphuration is performed 1) in an actual unit of the process with the aid of the feed to be treated in the presence of hydrogen and of hydrogen sulphide ( $H_2S$ ) introduced as is or as the degradation product of an organic sulphur compound, this being called sulphuration in-situ or 2) before the catalyst is fed into the unit, called sulphuration ex-situ. In the case of sulphuration ex-situ, mixtures of gases may be advantageously implemented, such as the mixtures  $H_2/H_2S$  or  $N_2/H_2S$ . The catalyst in its oxide form may also be advantageously sulphured ex-situ starting with model compounds in the liquid phase, the sulphuring agent then being selected from dimethyl disulphide (DMDS), dimethyl sulphide, n-butyl mercaptan, the polysulphide compounds of the type tertionyl polysulphide, the latter being diluted in an organic matrix composed of aromatic or alkyl molecules.

Prior to the said sulphuration step, the said catalyst in its oxide form consisting of a mesostructured silicon oxide matrix comprising the said polyoxometalates trapped in its walls may be advantageously pretreated thermally according to methods well known to the person skilled in the art, preferably by calcination in air at a temperature within the range 300 to 1000°C. and preferably a temperature within the range 500 to 600°C. for a duration within the range 1 to 24 hours and preferably for a duration within the range 6 to 15 hours.

According to a preferred embodiment, the polyoxometalates trapped in the walls of the said mesostructured silicon oxide matrix may advantageously be partially or totally sulphured at the moment of the preparation method by direct synthesis of the said mesostructured silicon oxide matrix comprising the said polyoxometalates used according to the invention and preferably in the course of step b) of the said preparation method, by introducing into the solution, in addi-

tion to at least one surfactant, at least one polyoxometalate and at least one silica precursor, sulphured precursors advantageously selected from thiourea, thioacetamide, the mercaptans, the sulphides and the disulphides. Low-temperature degradation, that is, at a temperature within the range 80 to 90°C. of the said sulphur precursors, either during the maturation step c) or during the autoclaving step d) induces the formation of  $H_2S$ , thus enabling the sulphuration of the said polyoxometalates.

According to another preferred embodiment, the partial or total sulphuration of the said polyoxometalates may be advantageously carried out by introducing the said sulphurous precursors into step g) of partial or total regeneration of the said polyoxometalates trapped in the said mesostructured silicon oxide matrix of the catalyst used in the invention.

The catalyst implemented in the hydrodesulphuration process according to the invention may advantageously be used in any process known to the person skilled in the art enabling the desulphuration of hydrocarbon cuts, and preferably catalytic cracking gasoline cuts. The hydrodesulphuration process according to the invention may advantageously be implemented in any type of fixed-bed, moving-bed or bubbling-bed reactor. Preferably, the said hydrodesulphuration process is implemented in a fixed-bed reactor.

The invention is illustrated on the basis of the following examples.

## EXAMPLES

The examples which follow clarify the invention without, however, limiting the scope thereof.

### Example 1 (Non-Conforming)

#### Preparation of a Catalyst A1 of the Formulation CoMo Based on Cobalt and Molybdenum Deposited by Dry Impregnation of the Alumina Support with a Solution Containing the Corresponding Classical Molecular Precursors

The support used is a transition alumina having textural properties (specific surface area, pore volume, pore diameter) of (260 m<sup>2</sup>/g, 0.58 ml/g, 8.2 nm at the desorption maximum). The catalyst A1 is prepared according to the method consisting of a two-step impregnation of an aqueous solution prepared on the basis of ammonium heptamolybdate (NH<sub>4</sub>)<sub>6</sub>Mo<sub>7</sub>O<sub>24</sub> and cobalt nitrate Co(NO<sub>3</sub>)<sub>2</sub>·6H<sub>2</sub>O. A 2-hour drying step at 120°C. is performed as an intermediary measure between the two dry impregnations. Following a 2-hour maturation, the extrudates are dried at 100°C. overnight, then calcined in oxygen at 500°C. for 4 hours.

The catalyst A1 of the formulation CoMo, thus obtained in the oxide state, has a molybdenum content of 16.3 expressed in wt. % of oxide MoO<sub>3</sub> relative to the total mass of the catalyst and a cobalt content of 4.10 expressed in wt. % of oxide CoO, the percentages being expressed as percentage of oxide relative to the total mass of the catalyst. The molar ratio Co/Mo of this catalyst is 0.48.

Catalyst A1 has textural properties of specific surface area, pore volume and pore diameter of 210 m<sup>2</sup>/g, 0.48 ml/g, and 8 nm respectively. Catalyst A1 obtained was analysed by

21

Raman spectroscopy. No characteristic band of the presence of a heteropolyanion is detected.

Example 2 (Non-Conforming)

Preparation of a Catalyst A2 of the Formulation CoMoP Based on Cobalt, Molybdenum and Phosphorus Deposited by Dry Impregnation of the Alumina Support with a Solution Containing the Strandberg-Type Heteropolyanion of the Formula  $P_2Mo_5O_{23}^{6-}$

The support used is a transition alumina having textural properties of specific surface area, pore volume and pore diameter of  $260\text{ m}^2/\text{g}$ ,  $0.58\text{ ml/g}$ , and  $8.2\text{ nm}$  respectively. The catalyst A2 is prepared according to the method consisting of dry impregnation with an aqueous solution containing the Strandberg heteropolyanion of the formula  $P_2Mo_5O_{23}^{6-}$  the said heteropolyanion being obtained by solubilisation of molybdenum trioxide ( $MoO_3$ ) with orthophosphoric acid ( $H_3PO_4$ ) under reflux in stoichiometric proportions, and cobalt hydroxide  $Co(OH)_2$  is then added to the clear solution.

The volume of the solution containing the metal precursors is strictly equal to the pore volume of the support mass. The precursor concentrations of the aqueous solution are adjusted so as to deposit the desired contents by weight onto the support.

The Raman spectrum of the prepared solution clearly shows the characteristic bands of the Strandberg-type heteropolyanion.

The concentrations of precursor in the aqueous solution are adjusted so as to deposit the desired contents by weight on the support. The catalyst is then dried for 12 hours at  $120^\circ\text{C}$ .

Catalyst A2 thus obtained in the oxide state, of the formulation CoMoP, has a molybdenum content of 18% expressed in wt. % of molybdenum trioxide  $MoO_3$ , a cobalt content of 3.5 expressed in wt. % of cobalt oxide and a phosphorus content of 3.55 expressed in wt. % of oxide  $P_2O_5$ . The atomic ratio Co/Mo of this catalyst is 0.37 and the molar ratio P/Mo is 0.4. This catalyst does not conform to the invention.

The catalyst A2 has textural properties (specific surface area, pore volume, pore diameter) of ( $205\text{ m}^2/\text{g}$ ,  $0.42\text{ ml/g}$ ,  $8\text{ nm}$ ) respectively. This catalyst does not conform to the invention.

The catalyst obtained was analysed by Raman spectroscopy. This reveals an asymmetrical band at  $953$  and  $929\text{ cm}^{-1}$ , as well as the secondary bands at  $878$ ,  $399$ , and  $371\text{ cm}^{-1}$  characteristic of the Strandberg-type heteropolyanion  $P_2Mo_5O_{23}^{6-}$ , in agreement with the earlier results published by J. A. Bergwerff, T. Visser, B. R. G. Leliveld, B. D. Rossemaar, K. P. de Jong, and B. M. Weckhuysen, J. Am. Chem. Soc., 2004, 126, 44, 14548.

Example 3 (Non-Conforming)

Preparation of a Catalyst B1 of the Formulation CoMo Based on Cobalt and Molybdenum Deposited by Dry Impregnation of the Type SBA-15 Mesostructured Silica Support with a Solution Containing the Corresponding Classical Molecular Precursors

A type SBA-15 mesostructured silica material is synthesised in conformity with the teaching of the publication of D. Zhao, J. Feng, Q. Huo, N. Melosh, G. H. Frederickson, B. F. Chmelka, and G. D. Stucky, Science, 1998, 279, 548, in the following manner: 2 g F127 ( $PEO_{70}PPO_{106}PEO_{70}$ ) and 1.3 g

22

PPO (propylene polyoxide) are dispersed in 75 ml of an aqueous solution of 1.7 mol/l hydrochloric acid with agitation. 4.25 g tetraethyl orthosilicate ( $Si(OEt)_4$ , TEOS) is added to the homogeneous solution, and the whole is left under agitation at  $40^\circ\text{C}$ . for 24 hours. The suspension thus obtained is then poured into a 250-ml teflon autoclave and left at  $100^\circ\text{C}$ . for 24 hours. The solid is then filtered. The powder is then dried in air at  $100^\circ\text{C}$ ., then calcined at  $550^\circ\text{C}$ . in air for 4 h to degrade the copolymer and thus free the porosity. The solid has textural properties of specific surface area, pore volume, and pore diameter of  $450\text{ m}^2/\text{g}$ ,  $0.8\text{ ml/g}$ , and  $8\text{ nm}$  respectively.

The catalyst B1 is prepared according to the method which consists in dry impregnation with an aqueous solution prepared on the basis of ammonium heptamolybdate and cobalt nitrate, the volume of the solution containing the metal precursors being strictly equal to the pore volume of the support mass. The precursor concentrations of the aqueous solution are adjusted so as to deposit the desired contents by weight onto the support. The catalyst is then dried for 12 hours at  $120^\circ\text{C}$ ., and then calcined in air at  $500^\circ\text{C}$ . for 2 hours.

Catalyst B1 thus obtained in the oxide state, of the formulation CoMo, has a molybdenum content of 18 expressed in wt. % of oxide  $MoO_3$ , and a cobalt content of 4.2% expressed in wt. % of oxide  $CoO$ . The atomic ratio Co/Mo of this catalyst is 0.45. This catalyst does not conform to the invention.

The isothermic analysis of nitrogen adsorption reveals a BET surface area of  $360\text{ m}^2/\text{g}$  for a pore volume of  $0.62\text{ ml/g}$  with a mean pore diameter of  $9.1\text{ nm}$ . This catalyst does not conform to the invention.

Example 4 (Non-Conforming)

Preparation of a Catalyst B2 of the Formulation CoMoP Based on Cobalt, Molybdenum and Phosphorus Deposited by Dry Impregnation of the Type SBA-15 Mesostructured Silica Support with a Solution Containing the Strandberg-Type Heteropolyanion of the Formula  $P_{21}Mo_5O_{23}^{6-}$

The type SBA-15 mesostructured silica material is synthesised as in Example 3. The solid obtained has the following textural properties and in particular a specific surface area, a pore volume and a pore diameter of  $450\text{ m}^2/\text{g}$ ,  $0.8\text{ ml/g}$ , and  $8\text{ nm}$  respectively. The catalyst B2 is prepared according to the method consisting of dry impregnation with an aqueous solution containing the Strandberg-type heteropolyanion of the formula  $P_2Mo_5O_{23}^{6-}$  obtained by solubilisation of molybdenum trioxide ( $MoO_3$ ) with orthophosphoric acid  $H_3PO_4$  under reflux in stoichiometric proportions, and of cobalt hydroxide  $Co(OH)_2$ .

The volume of the solution containing the metal precursors is strictly equal to the pore volume of the support mass. The precursor concentrations of the aqueous solution are adjusted so as to deposit the desired contents by weight onto the support.

The Raman spectrum of the prepared solution clearly shows the characteristic bands of the Strandberg-type heteropolyanion.

The concentrations of precursor in the aqueous solution are adjusted so as to deposit the desired contents by weight on the support. The catalyst is then dried for 12 hours at  $120^\circ\text{C}$ .

Catalyst B2 thus obtained in the oxide state, of the formulation CoMoP, has a molybdenum content of 18% expressed in wt. % of molybdenum trioxide  $MoO_3$ , a cobalt content of 3.7 expressed in wt. % of cobalt oxide and a phosphorus

content of 3.6 expressed in wt. % of oxide  $P_2O_5$ . The atomic ratio Co/Mo of this catalyst is 0.4 and the molar ratio P/Mo is 0.4. This catalyst does not conform to the invention.

The isothermic analysis of nitrogen adsorption reveals a BET surface area of  $356\text{ m}^2/\text{g}$  for a pore volume of  $0.6\text{ ml/g}$  with a mean pore diameter of  $9.0\text{ nm}$ . This catalyst does not conform to the invention.

The catalyst obtained was analysed by Raman spectroscopy. This reveals an asymmetrical band at  $952$  and  $928\text{ cm}^{-1}$ , as well as the secondary bands at  $877$ ,  $398$ , and  $370\text{ cm}^{-1}$  characteristic of the Strandberg-type heteropolyanion  $P_2Mo_5O_{23}^{6-}$ , in agreement with the earlier results published by J. A. Bergwerff, T. Visser, B. R. G. Lelieveld, B. D. Rossemaar, K. P. de Jong, and B. M. Weckhuysen, *J. Am. Chem. Soc.*, 2004, 126, 44, 14548.

#### Example 5 (Conforming to the Invention)

##### Preparation of a Catalyst C of the Formulation CoMoP Comprising the Strandberg-Type Heteropolyanion of Formula $P_2Mo_5O_{23}^{6-}$ trapped in a Type SBA-15 Mesostructured Silica Matrix

The SBA-15 mesostructured silica matrix comprising the Strandberg-type heteropolyanion of the formula  $P_2Mo_5O_{23}^{6-}$  trapped in its walls is obtained by direct synthesis according to the following method of preparation: the Strandberg-type heteropolyanion of the formula  $P_2Mo_5O_{23}^{6-}$  is obtained by solubilisation of molybdenum trioxide ( $MoO_3$ ) with orthophosphoric acid ( $H_3PO_4$ ) under reflux in stoichiometric proportions.

0.1 g of surfactant cetyltrimethylammonium bromide (CTAB) and 2.0 g of surfactant Pluronic P<sub>123</sub> (PEO<sub>20</sub>PPO<sub>70</sub>PEO<sub>20</sub>) are dissolved in 62.5 g of a 1.9 mol/l hydrochloric acid solution. 4.1 g of silica tetraethylorthosilicate (TEOS) precursor of the formula  $Si(OEt)_4$  is added, and then the medium is agitated for 45 min. 0.27 g of molybdenum trioxide  $MoO_3$  is solubilised in 0.07 g orthophosphoric acid  $H_3PO_4$  under reflux to obtain the Strandberg-type heteropolyanion of the formula  $P_2Mo_5O_{23}^{6-}$  in a solution 51. The solution 51 is then added to the mixture above. The colloidal solution obtained is then left under agitation for 20

hours at  $40^\circ\text{ C}$ . The suspension is decanted into a teflon autoclave for a treatment at a temperature of  $100^\circ\text{ C}$ . for 24 hours. The suspension thus obtained is filtered, then the solid, after washing with 30 ml of the 1.9 mol/l hydrochloric acid solution and 60 ml of distilled water, is dried overnight in the drying cupboard at  $40^\circ\text{ C}$ . The solid obtained is then calcined at a temperature level of  $490^\circ\text{ C}$ . for 19 hours in order to eliminate the surfactants and free the mesoporosity of the said solid.

10 The solid obtained is then introduced into an extractor of the Soxhlet type and the system is brought to reflux in the presence of methanol for 4 hours so as to partially regenerate the heteropolyanion partially degraded during the step of calcination. The solid is then dried to evacuate the solvent at a temperature of  $90^\circ\text{ C}$ . for 12 hours.

15 The solid obtained consisting of the SBA-15 mesostructured silica matrix comprising the Strandberg-type heteropolyanion of the formula  $P_2Mo_5O_{23}^{6-}$  trapped in its walls is then dry-impregnated with a solution of cobalt nitrate, then 20 dried at  $120^\circ\text{ C}$ . for 12 hours to evacuate the water. The final contents expressed in wt. % of oxides  $CoO$ ,  $MoO_3$  and  $P_2O_5$  are respectively  $3.6/18.0/3.55$  relative to the total mass of the catalyst. The atomic ratio Co/Mo of the catalyst C is 0.4 and the molar ratio P/Mo is 0.4. The catalyst C has the following 25 textural properties and in particular a specific surface area, a pore volume, and a pore diameter of  $348\text{ m}^2/\text{g}$ ,  $0.97\text{ ml/g}$ , and  $7.5\text{ nm}$  respectively and conforms to the invention.

20 The catalyst C obtained was analysed by Raman spectroscopy. This reveals an asymmetrical band at  $954$  and  $928\text{ cm}^{-1}$ , and secondary bands at  $877$ ,  $394$ , and  $370\text{ cm}^{-1}$  characteristic of the Strandberg-type heteropolyanion of the formula  $P_2Mo_5O_{23}^{6-}$ . The slight displacement of the bands of catalyst C as compared with a solution containing the heteropolyanion 30 with the support. The catalysts A1, A2, B1, C1, and C obtained in the examples 1, 2, 3, 4 and 5 are in powder form. In order to test these catalysts, they are first formed. For each example, the powders obtained are pelleted and then crushed. The catalysts are then tested in the form of particles of grain size within the range 1 and 2 mm.

35 Table 1 summarises the formulations of the catalysts, conforming and non-conforming to the invention.

TABLE 1

| Catalysts conforming and non-conforming to the invention. |                                                   |                                               |                                                   |                                               |                                                                      |
|-----------------------------------------------------------|---------------------------------------------------|-----------------------------------------------|---------------------------------------------------|-----------------------------------------------|----------------------------------------------------------------------|
|                                                           | A1<br>comparison                                  | A2<br>comparison                              | B1<br>comparison                                  | B2<br>comparison                              | C<br>conforms                                                        |
| support                                                   | alumina                                           | alumina                                       |                                                   | Silica SBA-15                                 |                                                                      |
| preparation                                               | Dry<br>impregnation                               | Dry<br>impregnation                           |                                                   | Dry impregnation                              | Trapping in the<br>matrix                                            |
| Precursors                                                | ammonium<br>heptamolybdate +<br>cobalt<br>nitrate | $P_2Mo_5O_{23}^{6-}$ +<br>cobalt<br>hydroxide | ammonium<br>heptamolybdate +<br>cobalt<br>nitrate | $P_2Mo_5O_{23}^{6-}$ +<br>cobalt<br>hydroxide | $P_2Mo_5O_{23}^{6-}$ +<br>cobalt<br>nitrate<br>post-<br>impregnation |
| $MoO_3$ wt. %                                             | 16.3                                              | 18                                            | 18                                                | 18                                            | 18                                                                   |
| $CoO$ wt. %                                               | 4.1                                               | 3.5                                           | 4.2                                               | 3.7                                           | 3.6                                                                  |
| $P_2O_5$ wt. %                                            | —                                                 | 3.55                                          | —                                                 | 3.6                                           | 3.55                                                                 |
| Co/Mo                                                     | 0.48                                              | 0.37                                          | 0.45                                              | 0.4                                           | 0.38                                                                 |
| P/Mo                                                      | —                                                 | 0.40                                          | —                                                 | 0.40                                          | 0.40                                                                 |
| SBET $\text{m}^2/\text{g}$                                | 210                                               | 205                                           | 360                                               | 356                                           | 348                                                                  |
| VPT* (ml/g)                                               | 0.48                                              | 0.42                                          | 0.62                                              | 9                                             | 7.5                                                                  |
| dp* mean<br>(nm)                                          | 8                                                 | 8                                             | 9.1                                               | 18                                            | 18                                                                   |

25

## Example 7

## Comparison of the Test Catalysts on Actual Feeds

The catalysts previously described were compared in the hydrodesulphuration of a gasoil derived by direct distillation.

The principal characteristics of the feed are given below:

Density at 15° C.: 0.8484

Sulphur: 1.21 wt. %

Simulated distillation:

PI: 165° C.

10%: 253° C.

50%: 308° C.

90%: 370° C.

PF: 409° C.

The test is conducted in an isothermal pilot reactor on a current-carrying stationary bed, the fluids circulating against gravity. After sulphuration in situ at 350° C. in the unit under pressure by means of the gasoil to which 2 wt. % of dimethyl disulphide has been added, the hydrodesulphuration was conducted under the following operating conditions:

Ratio H<sub>2</sub>/HC: 400 l/l

Total pressure: 7 MPa

Catalyst volume: 40 cm<sup>3</sup>

Temperature: 340° C.

Hydrogen flow rate: 32 l/h

Flow rate of feed: 80 cm<sup>3</sup>/h

Hourly space velocity: 2 h<sup>-1</sup>.

The catalytic performances of the catalysts under test are shown in the table below. They are expressed in relative activity, positing that that of the catalyst A1 is equal to 100 and considering that they are of the order of 1.5. The equation linking the activity and the hydrodesulphuration conversion (% HDS) is the following:

$$A_{HDS} = \frac{100}{[(100 - \% HDS)]^{0.5}} - 1$$

TABLE 2

| Activity of the catalysts in gasoil hydrodesulphuration |                                                                                                                               |                                 |
|---------------------------------------------------------|-------------------------------------------------------------------------------------------------------------------------------|---------------------------------|
| Catalyst                                                |                                                                                                                               | <sup>4</sup> HDS relative to A1 |
| A1<br>(reference)                                       | CoMo/Al <sub>2</sub> O <sub>3</sub>                                                                                           | 100                             |
| A2<br>(non-conforming)                                  | CoMoP (P <sub>2</sub> Mo <sub>5</sub> O <sub>23</sub> <sup>6-</sup> + cobalt hydroxide)/Al <sub>2</sub> O <sub>3</sub>        | 110                             |
| B1<br>(non-conforming)                                  | CoMo/mesostructured SiO <sub>2</sub>                                                                                          | 52                              |
| B2<br>(non-conforming)                                  | CoMoP (P <sub>2</sub> Mo <sub>5</sub> O <sub>23</sub> <sup>6-</sup> + cobalt hydroxide)/mesostructured SiO <sub>2</sub>       | 75                              |
| C<br>(conforming)                                       | CoMoP (P <sub>2</sub> Mo <sub>5</sub> O <sub>23</sub> <sup>6-</sup> then cobalt nitrate) trapped in the mesostructured silica | 115                             |

Impregnation of a solution containing the Strandberg-type heteropolyanion of the formula P<sub>2</sub>Mo<sub>5</sub>O<sub>23</sub><sup>6-</sup> onto an alumina support (catalyst A2, non-conforming) enables the activity of a catalyst to be improved relative to the reference catalyst A1.

Use of a type SBA15 mesoporous silica, without particular preparation precautions, that is to say, by impregnating onto the said silica a solution containing the precursors of cobalt

26

and molybdenum, leads to an almost 50% decline in activity (catalyst B1, non-conforming) relative to the reference catalyst A1.

Impregnation onto this same silica of a solution containing the Strandberg-type heteropolyanion of the formula P<sub>2</sub>Mo<sub>5</sub>O<sub>23</sub><sup>6-</sup> (catalyst B2, non-conforming) enables the activity to be increased relative to non-conforming catalyst B1, although without achieving that of the reference catalyst A1.

Finally, the fact of trapping the active phase, in the form of a Strandberg-type heteropolyanion of the formula P<sub>2</sub>Mo<sub>5</sub>O<sub>23</sub><sup>6-</sup> (catalyst C, conforms) enables the activity to be greatly increased relative to the reference catalyst A1 and an improved activity to be achieved relative to the other non-conforming catalysts of the prior art.

## Example 8

## Comparison of the Test Catalysts of Hydrogenation of an Aromatic Model Molecule Feed

The catalysts described above are sulphured in situ under dynamic conditions in a tubular reactor with a current-carrying stationary bed, the fluids circulating from top to bottom. The hydrogenating activity measurements are carried out immediately after the sulphuration under pressure without re-exposure to air, with the hydrocarbon feed used to sulphurise the catalysts.

The sulphuration test feed was composed of 5.8% dimethyl disulphide (DMDS), 20% toluene and 74.2% cyclohexane (by weight).

Thus the stabilised catalytic activities were measured in the toluene hydrogenation reaction.

The activity measuring conditions are as follows:

Total pressure: 6.0 MPa  
Pressure of toluene: 0.38 MPa  
Pressure of cyclohexane: 1.55 MPa  
Pressure of hydrogen: 3.64 MPa  
Pressure of H<sub>2</sub>S: 0.22 MPa  
Catalyst volume: 40 cm<sup>3</sup>  
Flow rate of feed: 80 cm<sup>3</sup>/h  
Hourly space velocity: 21/l/h<sup>-1</sup>  
Hydrogen flow rate: 36 l/h  
Sulphuration and test temperature: 350° C. (ramping of 3° C./min).

Samples of the liquid effluent were analysed by gas chromatography. Determination of the molar concentrations in unconverted toluene (T) and concentrations of the products of hydrogenation (methylcyclohexane (MCC6), ethylcyclopentane (EtCC5) and the dimethylcyclopentanes (DMCC5)) enable calculation of the rate of toluene hydrogenation XHYD, defined by:

$$X_{HYD}(\%) = 100 * \frac{(MCC6 + EtCC5 + DMCC5)}{(T + MCC6 + EtCC5 + DMCC5)}$$

With the toluene hydrogenation reaction of order 1 under the implemented test conditions, and the reactor behaving like an ideal piston reactor, the hydrogenating activity AHYD of the catalysts is calculated by applying the formula:

$$AHYD = \ln(100/(100 - X_{HYD}))$$

Table 3 compares the relative hydrogenating activities, equal to the ratio of the activity of the catalyst under consideration to the activity of the catalyst A1 taken as the reference (activity 100%).

TABLE 3

| Catalyst               |                                                                                                                               | AHYD for iso-volume of catalyst relative to A1 |
|------------------------|-------------------------------------------------------------------------------------------------------------------------------|------------------------------------------------|
| A1<br>(reference)      | CoMo/Al <sub>2</sub> O <sub>3</sub>                                                                                           | 100                                            |
| A2<br>(non-conforming) | CoMoP (P <sub>2</sub> Mo <sub>5</sub> O <sub>23</sub> <sup>6-</sup> + cobalt hydroxide)/Al <sub>2</sub> O <sub>3</sub>        | 190                                            |
| B1<br>(non-conforming) | CoMo/mesostructured SiO <sub>2</sub>                                                                                          | 80                                             |
| B2<br>(non-conforming) | CoMoP (P <sub>2</sub> Mo <sub>5</sub> O <sub>23</sub> <sup>6-</sup> + cobalt hydroxide)/mesostructured SiO <sub>2</sub>       | 110                                            |
| C<br>(conforming)      | CoMoP (P <sub>2</sub> Mo <sub>5</sub> O <sub>23</sub> <sup>6-</sup> then cobalt nitrate) trapped in the mesostructured silica | 130                                            |

Table 3 shows the large gain in hydrogenating activity relative to iso-volume that is obtained on the catalysts prepared on the basis of impregnation of a solution containing the Strandberg-type heteropolyanion of the formula P<sub>2</sub>Mo<sub>5</sub>O<sub>23</sub><sup>6-</sup> (catalyst A2 by comparison with the reference catalyst A1).

The toluene hydrogenation activity of the toluene develops in the majority of cases in parallel with the hydrodesulphuration activity. It is similarly representative of hydrogenation of the aromatic compounds, and thus of the hydrogen consumption induced by the catalyst in question.

In the case of the catalyst C conforming to the invention, it should be noted that, as shown in Table 2, the hydrodesulphuration activity is greater than that of the reference catalyst A1, and that of the catalyst A2, whereas the toluene hydrogenation activity is inferior to that of the catalyst A2, making it possible to predict a moderate hydrogen consumption for the catalysts conforming to the invention.

The invention claimed is:

1. A hydrodesulphuration process of at least one gasoil cut implementing a catalyst comprising, in its oxide form, at least one metal from group VIB and/or at least one metal from group VIII of the periodic table present in the form of at least one polyoxometalate, which is

an Anderson heteropolyanion of formula XM<sub>6</sub>O<sub>24</sub><sup>q-</sup>,

a Keggin heteropolyanion of formula XM<sub>12</sub>O<sub>40</sub><sup>q-</sup>,

a lacunary Keggin heteropolyanion of formula XM<sub>11</sub>O<sub>39</sub><sup>q-</sup>, or

a Strandberg heteropolyanion of formula H<sub>h</sub>P<sub>2</sub>Mo<sub>5</sub>O<sub>23</sub><sup>(6-h)-</sup>,

wherein

X is an element selected from the group consisting of phosphorus (P), silicon (Si), boron (B), nickel (Ni) and cobalt (Co), the said element being taken alone,

M is one or more element(s) selected from the group consisting of molybdenum (Mo), tungsten (W), nickel (Ni) and cobalt (Co),

O is oxygen,

H is hydrogen,

h is an integer in the range 0 to 12, and

q is an integer in the range 1 to 20,

the said polyoxometalates being present within a meso-

structured silicon oxide matrix having a pore size within the range 1.5 to 50 nm and having amorphous walls of thickness within the range 1 to 30 nm, the said catalyst being sulphured before being implemented in the said process.

2. A process according to claim 1, wherein the gasoil cut is a cut at least 90% of the compounds of which have a boiling point within the range 250° C. to 400° C.

3. A process according to claim 1, wherein the gasoil cut is selected from the group consisting of gasoil cuts derived by direct distillation, alone or in admixture with at least one cut derived from a coking unit, at least one cut derived by catalytic cracking, and at least one gasoil cut derived from hydrocracking or residue hydrotreatment.

4. A process according to claim 1, wherein the polyoxometalate is an Anderson heteropolyanion of formula XM<sub>6</sub>O<sub>24</sub><sup>q-</sup>.

5. A process according to claim 1, wherein the polyoxometalate is a Keggin heteropolyanion of formula XM<sub>12</sub>O<sub>40</sub><sup>q-</sup>.

6. A process according to claim 5, wherein the Keggin heteropolyanion is of formula PMo<sub>12</sub>O<sub>40</sub><sup>3-</sup>, and additionally present are cations 3H<sup>+</sup>, whereby the catalyst contains a heteropolyacid of formula PMo<sub>12</sub>O<sub>40</sub><sup>3-</sup>, 3H<sup>+</sup>.

7. A process according to claim 1, wherein the polyoxometalate is a Strandberg heteropolyanion of formula H<sub>h</sub>P<sub>2</sub>Mo<sub>5</sub>O<sub>23</sub><sup>(6-h)-</sup>.

8. A process according to claim 1, wherein said catalyst in its oxide form exhibits a form of each of the elementary particles of which it is composed that is non-spherical.

9. A process according to claim 1, wherein the catalyst comprises a content of the group VIB element by weight, expressed as wt. % of oxide relative to the total mass of the catalyst, in the range of 1 to 30 wt. %.

10. A process according to claim 1, wherein the catalyst comprises a content by mass of the group VIII element expressed in percentage by weight of oxide relative to the total mass of the catalyst in the range of 0.1 to 10 wt. %.

11. A process according to claim 1, wherein the catalyst comprises a content by mass of doping element X selected from phosphorus, boron and silicon in the range of 0.1 to 10 wt. % of oxide relative to the final catalyst.

12. A process according to claim 1, wherein said process is implemented at a temperature in the range of 250° C. to 380° C., at a total pressure in the range of 2 MPa to 10 MPa with a ratio of the volume of hydrogen to volume of hydrocarbon feed in the range of 100 to 600 litres per litre, and at an hourly space velocity (HSV) defined by the ratio of the volumetric flow rate of liquid hydrocarbon feed to the volume of catalyst fed into the reactor in the range of 1 to 10 h<sup>-1</sup>.

13. A process according to claim 1, wherein the polyoxometalate is a lacunary Keggin heteropolyanion of formula XM<sub>11</sub>O<sub>39</sub><sup>q-</sup>.

\* \* \* \* \*